

Jan. 22, 1935.

R. SCHMIDT

1,988,812

SOUND NEGATIVE FOR DIRECT PRODUCTION OF SOUNDS

Filed July 28, 1932

Fig. 1

density curve



Fig. 2

transparency curve



Inventor:  
Richard Schmidt,  
By Philip S. Hopkins,  
Attorney.

## UNITED STATES PATENT OFFICE

1,988,812

## SOUND NEGATIVE FOR DIRECT PRODUCTION OF SOUNDS

Richard Schmidt, Dessau, Germany, assignor to  
 Agfa Ansco Corporation, Binghamton, N. Y., a  
 corporation of New York

Application July 28, 1932, Serial No. 625,515  
 In Germany August 1, 1931

1 Claim. (Cl. 95—5)

My present invention relates to the manufacture of photographically registered sound records and more particularly to the manufacture of such records produced according to the varying density method.

One of its objects is to provide a process according to which sound negatives are obtainable for direct use without their printing being necessary. Another object is the sound negatives giving directly a true reproduction of the original sounds. Further objects will be seen from the detailed specification following hereafter. Reference is made to the accompanying drawing showing in Fig. 1 the density and in Fig. 2 the transparency curve of a silver halide gelatin emulsion well suited for the production of such sound negatives.

I have found that by a suitable development sound negatives, produced according to the varying density method, are obtainable which give a true or substantially true reproduction of the tonal values and which may be used for direct sound reproduction. In order to realize this problem development must be effected in such a manner that the curve of transparency, i. e. the curve determined by the values of  $it$  (light intensity multiplied by the time of exposure) as abscissæ and the transparencies  $T$  as ordinates is approximately a straight line. The density curve which is intimately related to the transparency curve and of which the abscissæ are graduated in values of  $\log it$  ( $it$ =light intensity multiplied with the time of exposure) and the ordinates in values of density  $s$  should approach as nearly as possible a logarithmic curve. That means that the curve should be very flat in the region of weak blackenings and very steep for the region of blackenings beginning with densities  $s=0.5$  to 0.6. In order to permit the registration of a great intensity range the straight region of the transparency curve should be as long as possible.

For this purpose a suitable silver halide emulsion must be selected and it has been found that the emulsions which are most suitable for the present invention are those that have hitherto been used for the production of aerial surveys. It is first necessary to make a record of the transparency curve of this emulsion in order to determine the intensity of light which must be used in making the sound record. The value of the abscissa in the middle of the straight portion of the transparency curve gives the intensity of light required. After exposure, the emulsion containing the sound record is developed by means of a so-called depth developer, preferably with a

developer such as is used for developing titles. Such developers yield clean negatives showing great contrasts.

As known, for the photographic registration of sounds there is used a source of light of which in the varying density method, the intensity is changed in accordance with the sound waves to be registered. That means according to the oscillations of the sound waves the intensity of the source of light varies around a mean value which corresponds with the light intensity when the sound recording apparatus is at rest. This mean value is given the mean value of the abscissæ of the straight part of the transparency curve.

For better understanding I will now describe my invention with reference to the accompanying drawing.

In Fig. 1 there is shown a density curve of a silver halide gelatin emulsion suited for the production of a sound negative for direct reproduction of the original sounds. The values for tracing this curve have been ascertained in an "ultra-short-time" sensitometer realizing the conditions usual in taking a sound negative. In determining this curve one of the factors must be constant, in the present case the time of exposure is of the product  $\log it$  chosen as the constant factor and has been given about 1/22000 sec. the time used in taking a sound record varying generally in the range of 1/20000 sec. to 1/30000 sec. and being determined by the speed at which the film is fed through the apparatus and the breadth of the slit. The change of intensity of the source of light used for exposing the film was effected by interposition of a blackened wedge. The exposed film, in the present case "Aero-chromfilm" (Agfa), was developed for about 10 minutes in a developer as usual for title developing. In the figure  $ab$  designates that part of the curve which is applicable for the production of sound negatives giving directly a true reproduction of the original sounds without the necessity for a printing process.

In Fig. 2 there is shown the transparency curve corresponding with the density curve shown in Fig. 1. In this curve the part marked  $cd$  corresponds to the part  $ab$  of Fig. 1 and is useful for the purposes of the invention. It may be mentioned that the part applicable for the production of sound negatives according to this invention need not be an absolute straight line. A deviation of this condition is admissible so long as the limit given by a distortion of the upper harmonics is not crossed. The mean value of the light intensity to be used in taking

the sound record, that is the intensity of the source of light for exposing the film when the recording apparatus is in its rest position is given by the value of  $d$  corresponding in Fig. 5 2 with the abscissa 54 (the intensity units are arbitrary).

My invention is not limited to the foregoing example or to the specific details given therein. Changes in detail may occur to those skilled 10 in the art and I contemplate as included within my invention all such modifications as fall within the scope of the appended claims.

My invention is applicable to all kinds of cinematography concerned with sound recording, 15 but it is of particular importance for amateur cinematography, working with substandard film in which case for economy's sake no prints should be made. In the case of the reversal process, the sound record, after the simultaneous development of the picture and sound negative 20 is finished, is protected from further action of the treating liquids by providing it, in known manner, with a protective layer, whereupon the picture record is reversed to the positive in the

usual manner. Then after removal of the protective layer, the sound record is fixed. However, the sound track may also be provided with a protective layer before beginning the treatment of the picture area and after the pictures have been produced, the protection layer is removed and the sound record is developed and fixed in the manner above described.

What I claim is:—

The process of producing a sound negative 10 adapted for direct reproduction of the sound which comprises exposing a film of steep gradation to a source of light having its intensity varying with sound waves to be recorded, adjusting the intensity of the unmodulated source of 15 light to the mean value of the abscissæ of the straight part of the transparency curve if said film the abscissæ designating it (light intensity multiplied by the time of exposure) wherein  $t$  has a constant value and substantially corresponds with the period of exposure used in recording, and developing the exposed film to a steep gradation.

RICHARD SCHMIDT.